

Dec. 26, 1922.

1,439,683.

R. F. BACON ET AL.  
MANUFACTURE OF GASOLINE.  
FILED OCT. 19, 1914.



Inventors  
Raymond F. Bacon  
Benjamin J. Brooks  
Attorneys  
Penrie Davis Morris  
By their

## UNITED STATES PATENT OFFICE.

RAYMOND F. BACON AND BENJAMIN T. BROOKS, OF PITTSBURGH, PENNSYLVANIA,  
ASSIGNORS TO GULF REFINING COMPANY, OF PITTSBURGH, PENNSYLVANIA, A  
CORPORATION OF TEXAS.

## MANUFACTURE OF GASOLINE.

Application filed October 19, 1914. Serial No. 867,429.

To all whom it may concern:

Be it known that we, RAYMOND F. BACON and BENJAMIN T. BROOKS, residing at Pittsburgh, State of Pennsylvania, have invented 5 certain new and useful Improvements in the Manufacture of Gasoline; and we do hereby declare the following to be a full, clear, and exact description of the invention, such as will enable others skilled in the art to which 10 it appertains to make and use the same.

In Letters Patent of the United States granted to us jointly with Clinton W. Clark, No. 1,131,309, is described the treatment of mineral oils for the production of a mixture of hydrocarbons, principally of the  $C_nH_{2n+2}$  series, boiling below 200° C. This product may be conveniently designated as gasoline or light petroleum distillates, suitable for use in internal combustion engines 15 and is intended principally for such use.

The present invention is based upon the discovery that when working under like conditions of temperature and pressure to those specified in the patent referred to, 20 greater yields of gasoline are obtained by using, as the charge for the still, the hereinafter described heavier part of the distillate from crude petroleum, instead of either the whole distillate boiling above approximately 150° C., or instead of a reduced crude containing considerable proportions of asphaltic matter; and, furthermore, that, in such case, there is a considerable decrease in the amount of coke produced in 25 the gasoline-making operation.

In the ordinary fractional distillation of crude petroleum (for instance, "Oklahoma crude" or "mixed base"), the fraction distilled off between the kerosene and the lightest lubricating oil cuts is known as "solar oil" and has a specific gravity (e. g., of about 0.86) and viscosity less than said lightest lubricating oils. We have found that this solar oil fraction is of relatively 40 low capacity as a crude material for the production of gasoline. For instance, in treating solar oil obtained from Oklahoma crude, the yield of gasoline, at a pressure of 100 pounds to the square inch and a temperature of 400° C., is from 8 to 10% of the charge; whereas, when Oklahoma crude oil from which the gasoline originally contained in the oil is removed is treated under

the same conditions of pressure and temperature there is a yield of 18 to 20% of 55 the charge. Still further, when the lighter fractions and the solar oil have first been fractionally distilled off from the crude oil and the heavy distillate substantially free from the heavy base constituents of the 60 petroleum whose employment is characteristic of the present invention is collected separately and treated under the same conditions of pressure and temperature the yield of gasoline was found to rise to from 28 65 to 30% of the heavy distillate charge. This unexpected and radical increase in yield of gasoline under like conditions of treatment could not have been predicted from any information possessed by those skilled in 70 the art, and constitutes an improvement of corresponding value and importance.

Referring further to the "heavy distillate" which constitutes the material treated for the production of gasoline in accordance 75 with the present invention, it may be said that it has the specific gravity and typical greasiness or viscosity of lubricating oil, namely, a specific gravity between 0.860, and about 0.960, and a mean value of about 0.875 80 to 0.920, and a viscosity of 5° to 15° Engler. This heavy distillate (if from "Oklahoma crude") is made up for the most part of liquid naphthenes and polynaphthenes of unsaturated hydrocarbons liquid at ordinary 85 temperature belonging to the unsaturated series,  $C_nH_{2n}$   $CnH_{2n-2}$ ,  $CnH_{2n-4}$ . In the trade, it is known sometimes as crude lubricating distillate, and may or may not contain paraffine, but, being a distillate, it is substantially free from heavy residuum or base constituents. The presence of paraffine, the exact specific gravity, the color, and the like, will vary somewhat in individual instances, within limits recognized in the art. 90 However, a typical crude oil will yield by ordinary distillation processes, say 40% of gasoline and kerosene, about 30% of solar oil, and finally about 25% of the heavy oil referred to herein as "heavy distillate." 95

In carrying out the invention, we prefer, as hereinbefore indicated, to employ the same range of temperatures and the same pressures that characterize the treatment set forth in the patent referred to, and, indeed, the same apparatus may be employed 100 105

to advantage, all as hereinafter more fully set forth. We have obtained satisfactory yields with pressures as low as 60 pounds to the square inch, and, while the yield increases at higher pressures, we do not ordinarily find it of advantage to increase the pressure absolutely to the upper limit of 300 pounds; in fact, there is usually no such material advantage in yield in raising the pressure above say 250 pounds as would compensate for the increased expense of so doing. Indeed, for safety of operation, it will suffice ordinarily to conduct the operation at a pressure of say 100 to 150 pounds per square inch, and at a temperature ranging from 350° C. to 500° C.

While we recommend the general form of apparatus shown in the accompanying drawing as appropriate to the practice of the invention, it will, of course, be understood that we do not limit ourselves thereto, inasmuch as the characteristic feature of the invention consists in the discovery hereinbefore carefully pointed out, to wit, that by employing the heavy distillate referred to a greater proportion of the complex hydrocarbons are cracked up into the simpler gasoline hydrocarbons, under the same conditions of pressure and temperature, and that this increased yield in the desired product is likewise accompanied by a diminished deposit of coke in the pressure still.

It will, of course, be understood that the optimum results obtainable are produced when solar oil is substantially absent from the heavy distillate, inasmuch as solar oil yields proportionately less gasoline. In practice, however, a certain minor amount of solar oil may nevertheless be tolerated in the heavy distillate without seriously interfering with the percentage yield and, indeed, in some of the so-called paraffine distillates a notable quantity of solar oil is present, say, in some instances, up to 10 to 15%. The treatment of such a distillate we regard as within the broad scope of our invention. While we do not recommend that, in any case, the amount of solar oil shall exceed that percentage, we prefer that its percentage be as low as is economically feasible.

In the accompanying drawing, Figure 1 represents, partly in section, and partly in elevation, a form of apparatus suitable for the practice of the invention; Fig. 2 represents a partial view of another modification of the invention, showing its applicability to advantage in multiple units.

Similar letters of reference indicate similar parts in both the views.

Referring particularly to Fig. 1, A indicates a storage tank for the petroleum hydrocarbons to be treated, and B indicates a pump for delivering a regulated supply therefrom to the still through the conduit a.

In Fig. 1, is shown a single unit consisting

of a tube b, of steel or other suitable metal and whose length is preferably 20 ft. or more, when the internal diameter of the tube is 6 inches. The heating zone of the tube is intermediate of its ends and, in the form shown in Fig. 1, consists of a fire brick chamber C having suitable air inlets, as d, and a suitable exit opening, as e, for the products of combustion. The chamber C may receive its heat from any convenient source, as, for instance, a series of annular gas burners, f, supplied with a mixture of air and gas from the gas conduit D whose branches g terminate in injecting tips, as shown, and which draw in with them a suitable supply of air through the bell h opening into the atmosphere. At its lower end, the tube b communicates with a tar and coke receiving receptacle E, located below, outside of the heating zone.

At the beginning of the operation, the charge of oil to be cracked and distilled is established up to the level indicated in Fig. 1, that is to say, at a level slightly higher than the internal wall of the top of the heating chamber C. This level of the body of oil is kept practically constant, by means of the pump B, which supplies oil to the interior of the tube as the cracking and distillation proceed. Accordingly, the products of combustion do not come into direct contact with any portions of the tube not occupied by the liquid oil, and consequently, the danger of destructive distillation of any portion of the vapors by coming into contact with overheated portions of the tube above the zone of liquid oil is minimized and the formation of an adhering layer of coke upon such portion of the walls of the tube is avoided.

The free portion of the tube extends above the furnace setting, as shown, for a distance of say 5 feet. The vapors pass, by means of the pipe i, to the condenser coil J, contained within the cooling receptacle F. The condenser coil is provided at its end with a valve k and discharges into the receptacle G. The uncondensed gases and vapors from the receptacle G pass by the pipe l into a body of oil contained within the receptacle H, wherein such particles of oil as are contained in the residual gases are trapped and recovered. The surplus gases and vapors pass off through the conduit m. At the bottom of the receptacle E a pipe n conveys the residual tar and coke to a receiving tank I, the flow being under the control of a regulable valve s.

From the foregoing description of the purposes of the invention, and of the construction of the apparatus shown in Fig. 1, the mode of operation will be fully apparent. The receptacle E and the tube B, are filled to the level indicated, and the annular burners f are ignited. The tempera-

ture rises to the range hereinbefore referred to, that is to say, 350° C. to 500° C., and the pressure is likewise permitted to rise, by shutting off the valve K either wholly or 5 partially, as the case may be, until the pressure gage  $\ell$  indicates the pressure desired, that is to say, a pressure within the range of 60 lbs. to 300 lbs. per square inch.

During the cracking and distilling operation, any particles of tar and coke that may be formed in the body of the distilling oil tend to fall through the vertical heating zone, by gravity, into the receiving space of the chamber E. A relatively small 10 amount of tar and coke will, in the course of time, build up upon the vertical walls of the tube B within the heating zone, but these accumulations are relatively unimportant and slow of formation, and, should 15 they become excessive, may be readily removed by the use of any ordinary boiler flue cleaner, or the like. The petroleum residue containing the coke accumulating in the receptacle E is drawn off from time to 20 time through the pipe  $n$  into the receiver I.

In the form of the invention indicated in Fig. 2, there is shown a series of individual tubes  $b$ , having at the bottom a common header E' corresponding in function and 25 location to the receptacle E of Fig. 1. The tubes  $b$  are located in a heating flue C' supplied with a flow of hot products of combustion from any suitable source, so as to heat the tubes to the high temperatures hereinbefore referred to, the header E' being located in a cooler space below the heating flue.  $a'$  indicates a supply pipe communicating with the interior of the several tubes  $b$ , so as to furnish oil thereto. So also, the 30 pipe  $i'$  constitutes the exit pipe for the vapors. The supply pipe  $a'$  and the exit pipe  $n'$  from the header E' are connected by the cross-connecting pipe  $v$  having a valve  $x$  and containing the liquid level gage  $w$ , 35 so that the operator will be able to know at any time the oil level within the several tubes  $b$ . The mode of operation of this modification will be clear from what has been said in regard to the mode of operation 40 of the form of the apparatus shown in Fig. 50 1, and need not be further elaborated.

What we claim is:

1. The method of producing from petroleum oils containing asphaltic base constituents a product intended particularly for use as fuel for internal combustion engines, which consists in subjecting a heavy distillate of such petroleum having a specific gravity above 0.860 and which is substantially free from lower boiling solar oil having a specific gravity of about 0.860 and below, and which is also substantially free from heavy base constituents of the petroleum, to a combined cracking and distilling operation at a pressure within the range of 60

pounds to 300 pounds per square inch, and at a temperature within the range of 300° C. to 500° C.

2. The method of producing from petroleum oils containing asphaltic base constituents a product intended particularly for use as fuel for internal combustion engines, which consists in subjecting a heavy distillate of such petroleum containing a considerable proportion of naphthene hydrocarbons, 70 said distillate being substantially free from the lower boiling oil having a specific gravity of about 0.860 and below, and said distillate being also substantially free from heavy base constituents of the petroleum, to 75 a combined cracking and distilling operation at a pressure within the range of 60 pounds to 300 pounds per square inch, and at a temperature within the range of 300° C. to 500° C.

3. The method of producing from petroleum oils a product intended particularly for use as fuel for internal combustion engines, which consists in subjecting a heavy distillate of mixed base petroleum, which 90 heavy distillate has a specific gravity of above 0.860 and is substantially free from the lower boiling solar oil having a specific gravity of 0.860 and below, and is also substantially free from heavy base constituents of the 95 petroleum to a combined cracking and distilling operation, at a pressure within the range of 60 pounds to 300 pounds per square inch and at a temperature within the range of 300° C. to 500° C.

4. The method of producing from petroleum oils containing asphaltic base constituents a product intended particularly for use as fuel for internal combustion engines, which consists in subjecting a heavy distillate of such petroleum having a specific 100 gravity above 0.860 and which is substantially free from the lower boiling solar oil having a specific gravity of about 0.860, and below, and which is also substantially free from heavy base constituents of the petroleum, to a combined cracking and distilling operation, at a pressure within the range of 60 pounds to 300 pounds per square inch, and at a temperature within the range of 105 300° C. to 500° C. progressively removing from the cracking and distilling zone the particles of tar and coke reduced therein and depositing them out of contact with the walls of the cracking and distilling zone.

5. The method of producing from petroleum oils a product intended particularly for use as fuel for internal combustion engines, which consists in subjecting a heavy distillate of mixed base petroleum, which 115 heavy distillate has a specific gravity above 0.860 and is substantially free from the low boiling solar oil having a specific gravity of 0.860 and below, and is also substantially free from heavy base constituents of the 120 125 130

- petroleum, to a combined cracking and distilling operation at a pressure within the range of 60 pounds to 300 pounds per square inch, and at a temperature within the range of 300° C. to 500° C. progressively removing from the cracking and distilling zone the particles of tar and coke produced therein, and depositing them out of contact with the walls of the cracking and distilling zone.
6. The method of producing from petroleum oils containing asphaltic base constituents a product intended particularly for use as fuel for internal combustion engines, which comprises separating from crude petroleum, containing such asphaltic base constituents a heavy distillate of specific gravity

above 0.860 and substantially free from base constituents and from lower boiling distillate having a specific gravity of 0.860 and below and subjecting said heavy distillate to a combined cracking and distilling operation at a pressure within the range of 60 pounds to 300 pounds per square inch, and at a temperature within the range of 300° C. to 500° C.

25

In testimony whereof we affix our signatures, in presence of two witnesses.

RAYMOND F. BACON.  
BENJAMIN T. BROOKS.

Witnesses:

H. H. SMITH,  
S. C. PERRING.

## DISCLAIMER

1,439,683.—*Raymond F. Bacon and Benjamin T. Brooks, Pittsburgh, Pa. MANUFACTURE OF GASOLINE.* Patent dated December 26, 1922. Disclaimer filed August 25, 1930, by the assignee, *Gulf Refining Company*.

Therefore disclaims from the scope or meaning of claims 1, 2, 3, 4, 5, and 6 of said Patent 1,439,683 any method of producing a product intended particularly for use as fuel for internal-combustion engines which includes subjecting petroleum oils to a pressure within a range below 100 pounds per square inch.

[*Official Gazette September 16, 1930.*]